

Patented Apr. 19, 1927.

## UNITED STATES PATENT OFFICE.

STANLEY FOWLER, OF YORKSHIRE, AND EDWIN EDSER, OF LONDON, ENGLAND.

## METHOD FOR THE PREVENTION OF CORROSION.

No Drawing. Original application filed April 26, 1926, Serial No. 104,833, and in Great Britain March 24, 1925. Divided and this application filed August 18, 1926. Serial No. 130,100.

This invention comprises improvements in or relating to methods for the prevention of corrosion.

We have discovered that if wool-fat is first rendered perfectly neutral and soap-free it can be brought into complete and permanent homogeneous union with oil, no sedimentation occurring, and that corrosion of metallic surfaces can be prevented very effectively by applying to them a covering layer of this clear homogeneous liquid, which we find is not the case to an equal extent with other preparations of wool-fat in non-volatile solvents.

According to the present invention therefore a method of preventing corrosion of metallic surfaces consists in covering the surface with a substantially non-acid layer consisting essentially of anhydrous neutral soap-free wool-fat in homogeneous unclouded admixture with a non-acid non-volatile thinning agent (for example a mineral-hydrocarbon such as mineral-lubricating oil).

The mixture of the pure neutral soap-free wool-fat and non-volatile thinning agent has moreover valuable properties as a lubricant and, when used for example for preventing corrosion of machined bearing-surfaces prior to assembly of machines, it is unnecessary to remove the protective layer before the parts are brought into use. The lubricant itself is the subject of our co-pending United States patent application Ser. No. 104,833 from which the present application is a divisional.

A method of preparing the wool-fat in a suitable state of particular purity is herein-after described. It is to be understood that wool-fat as ordinarily purified does not yield an unclouded solution free from sediment and is therefore unsuitable for use according to this invention.

In one method of carrying the invention into effect, pure neutral soap-free wool-fat is mixed with pure neutral mineral lubricating oil. The proportion of mineral oil may vary according to the consistency of the desired product. Mixing is done by pouring the molten purified wool-fat into the oil while stirring. The temperature of the mixture may reach 50° C. The amount of oil may be about three or more times the amount of wool-fat. If a less liquid product is desired, less mineral oil may be

added, or a thick mineral grease such as petroleum jelly may be used.

The composition is applied to articles which are to be protected from rust by any desired means, such as dipping, painting or spraying. It is found that the wool-fat imparts peculiar properties to the layer, rendering it strongly adherent notwithstanding the presence of the thinning agent so that it is not readily removed during handling, and yet the layer of the mixture is not gummy but possesses lubricating properties.

The wool-fat employed must be prepared in a way which renders it sufficiently neutral and soap-free and eliminates esters and other compounds which do not dissolve in mineral oils. One method is as follows:

The raw material is treated with alkali to effect saponification of the fatty acids contained in it, saponification being effected in successive stages with a quantity of alkali or the like in the initial stage or stages which is insufficient to effect complete saponification and the soaps produced at each stage being removed before proceeding to the next stage of saponification. It is found that emulsification of the wool-fat in the alkali, and consequent loss, is thus reduced. Two, three, or even four stages of saponification may be employed.

For example, crude wool-fat of the kind known as "white concentrate" (which separates from wool-washing effluent and forms a scum on the surface thereon when the effluent is allowed to stand) is run into a tank of boiling water at the rate of one and one half hundredweights of grease to 60 gallons of water, which is preferably soft. This is boiled for ten minutes. Cold water is then added in sufficient amount (about ninety gallons) to reduce the temperature to 46°

C. Assuming that the amount of fatty acid present is such that it would be neutralized by 22 ounces of sodium peroxide, twelve ounces of sodium peroxide are dissolved in 3 gallons of water and are added to the mixture with stirring. The whole is allowed to stand for twelve hours. It is then boiled to decompose any free sodium peroxide and to bring grease out of solution. It is allowed to settle and the aqueous portion is run off into a centrifugal machine, where the grease separates out and is returned to the original bulk.

The wool-fat (grease) is then washed by

boiling with 150 gallons of water, allowed to settle and the aqueous portion centrifuged as before. The centrifugally-separated wool-fat is again returned to the main bulk.

Into the grease is now mixed two-thirds of its bulk of water so as to be disseminated evenly therethrough. The temperature is adjusted to 46° C., and 10 ounces sodium peroxide are added, in solution as before, with stirring. This is allowed to stand for twelve hours, then diluted with 50 gallons of water and boiled. The aqueous portion only is decanted and centrifuged as before and the separated grease returned to bulk,

- 10 which is again washed by boiling with water, the aqueous portion is decanted and centrifuged and the recovered grease is returned to bulk. The product is the purified wool-fat. "Yorkshire brown grease" can be purified in the same way, using of course a greater quantity of alkali in view of the greater quantity of contained acids.

25 The product is then mixed with neutral mineral lubricating oil as above described, and is found to produce a clear solution free from cloudiness and sediment. The purified wool-fat yields less than 0.1% of ash and is therefore exceptionally free of soap, water and solid impurities and it contains less than 30 0.5% of fatty acid. Ordinary neutralised wool-fat contains notable percentages of soaps, while in wool-fat where soaps are absent there is usually present an objectionable amount of fatty acid or other bodies 35 which are insoluble in mineral oils. We have found that for the purpose of our invention it is essential to use wool-fat which is quite neutral, anhydrous and soap-free, if sedimentation is to be avoided on the one hand or injurious acid properties are to be

avoided on the other, and if effective prevention of corrosion is to be obtained. The wool-fat referred to in the claims is to be understood as being of the purity of that produced by the improved process set out above.

The process of producing this purified wool-fat, and the fat itself are claimed in our Patent No. 1,610,854, December 14, 1926, which was copending with this application, having been divided with this application from parent application Serial No. 104,833 filed April 26, 1926.

We claim:-

1. A method of preventing corrosion of 55 metallic surfaces which consists in covering the surface with a substantially non-acid layer consisting essentially of anhydrous neutral soap-free wool-fat in homogeneous unclouded admixture with a non-acid non-volatile thinning agent.

2. A method of preventing corrosion of metallic surfaces which consists in covering the surface with a substantially non-acid layer consisting essentially of anhydrous 65 neutral soap-free wool-fat in homogeneous unclouded admixture with a non-acid mineral-hydrocarbon.

3. A method of preventing corrosion of metallic surfaces which consists in covering 70 the surface with a substantially non-acid layer consisting essentially of anhydrous neutral soap-free wool-fat in homogeneous unclouded admixture with a non-acid mineral-lubricating oil.

In testimony whereof we affix our signatures.

STANLEY FOWLER.  
EDWIN EDSER.